

March 25, 1952

I. HARTER ET AL

2,590,311

PROCESS OF AND APPARATUS FOR CONTINUOUSLY CASTING METALS

Filed Feb. 26, 1948

10 Sheets-Sheet 1



Fig. 17

Isaac Harter  
Isaac Harter, Jr. &  
Otis R. Carpenter  
INVENTORS

Fig. 1

BY *J. P. Moran*  
ATTORNEY

March 25, 1952

I. HARTER ET AL

2,590,311

PROCESS OF AND APPARATUS FOR CONTINUOUSLY CASTING METALS

Filed Feb. 26, 1948

10 Sheets-Sheet 2



Isaac Harter  
Isaac Harter, Jr. &  
Otis R. Carpenter  
INVENTORS

BY *J.P. Moran*  
ATTORNEY

March 25, 1952

I. HARTER ET AL

2,590,311

PROCESS OF AND APPARATUS FOR CONTINUOUSLY CASTING METALS

Filed Feb. 26, 1948

10 Sheets-Sheet 3



Fig. 4



Fig. 12



Fig. 3



Isaac Harter  
Isaac Harter, Jr. &  
Otis R. Carpenter  
INVENTORS

BY *J.P. Moran*  
ATTORNEY

March 25, 1952

I. HARTER ET AL

2,590,311

PROCESS OF AND APPARATUS FOR CONTINUOUSLY CASTING METALS

Filed Feb. 26, 1948

10 Sheets-Sheet 4



Isaac Harter  
Isaac Harter, Jr.  
Otis R. Carpenter  
INVENTORS

BY *J. P. Moran*  
ATTORNEY

Fig. 6

March 25, 1952

I. HARTER ET AL

2,590,311

# PROCESS OF AND APPARATUS FOR CONTINUOUSLY CASTING METALS

Filed Feb. 26, 1948

10 Sheets-Sheet 5



Fig. 7



Fig. 8

*Isaac Harter  
Isaac Harter, Jr. &  
Otis R. Carpenter*  
INVENTORS

## INVENTORS

BY *J. Moran*  
ATTORNEY

**ATTORNEY**

March 25, 1952

I. HARTER ET AL

2,590,311

PROCESS OF AND APPARATUS FOR CONTINUOUSLY CASTING METALS

Filed Feb. 26, 1948

10 Sheets-Sheet 6



Isaac Harter  
Isaac Harter, Jr.  
Otis R. Carpenter  
INVENTORS

BY *J. Moran*  
ATTORNEY

March 25, 1952

I. HARTER ET AL

2,590,311

PROCESS OF AND APPARATUS FOR CONTINUOUSLY CASTING METALS

Filed Feb. 26, 1948

10 Sheets-Sheet 7



Fig. 13



Fig. 14



Fig. 15

Isaac Harter  
Isaac Harter, Jr. &  
Otis R. Carpenter  
INVENTORS

BY *J. P. Moran*  
ATTORNEY

March 25, 1952

I. HARTER ET AL

2,590,311

PROCESS OF AND APPARATUS FOR CONTINUOUSLY CASTING METALS

Filed Feb. 26, 1948

10 Sheets-Sheet 8



Fig. 16

Isaac Harter  
Isaac Harter, Jr.  
& Otis R. Carpenter  
INVENTORS

BY *J.P. Moran*  
ATTORNEY

March 25, 1952

I. HARTER ET AL

2,590,311

PROCESS OF AND APPARATUS FOR CONTINUOUSLY CASTING METALS

Filed Feb. 26, 1948

10 Sheets-Sheet 9

Fig. 18



Isaac Harter, Isaac Harter, Jr.  
& Otis R. Carpenter  
INVENTORS

BY *J. Moran*  
ATTORNEY

March 25, 1952

I. HARTER ET AL

2,590,311

PROCESS OF AND APPARATUS FOR CONTINUOUSLY CASTING METALS

Filed Feb. 26, 1948

10 Sheets-Sheet 10



Fig. 19

INVENTORS  
Isaac Harter  
BY Isaac Harter, Jr. &  
Otis R. Carpenter

J. P. Moran ATTORNEY

## UNITED STATES PATENT OFFICE

2,590,311

## PROCESS OF AND APPARATUS FOR CONTINUOUSLY CASTING METALS

Isaac Harter and Isaac Harter, Jr., Beaver, Pa., and Otis R. Carpenter, Barberton, Ohio, as signors, by mesne assignments, to The Babcock & Wilcox Company, Jersey City, N. J., a corporation of New Jersey

Application February 26, 1948, Serial No. 10,956

12 Claims. (Cl. 22—144)

1

The present invention relates in general to the continuous casting of metal products, and more particularly to a process of and apparatus for the continuous casting of ferrous metals and alloys in semi-finished and/or finished products of indeterminate length and various cross-sections.

The metals industry has long recognized the fact that a continuously cast semi-finished or finished product of acceptable commercial quality, whose length is limited solely by the amount of molten material available for pouring, offers considerable economic advantages inasmuch as it eliminates the metal casting losses due to cropping and scalping which occur in the production of ingots in individual stationary molds. Processes and apparatus have been in successful commercial use for years for the continuous casting of non-ferrous metals, such as copper and aluminum, having relatively low fusion temperatures and high thermal conductivities. Unwarranted claims have been made for many years in prior patents and publications of the applicability of apparatus and processes successfully developed for the continuous casting of these low fusion temperature metals to the continuous casting of ferrous and other high melting point alloy products. Yet in spite of the tremendous world production of, and demand for, steel and alloy steel products, for example, these prior apparatus and processes have heretofore failed to result in a single installation in commercial production for the continuous casting of steel and/or alloy steel products.

We believe that the inapplicability of the prior processes and apparatus successfully in use for the continuous casting of aluminum and copper to the continuous casting of steel is primarily due to the substantially different physical characteristics of carbon and alloy steels affecting the casting thereof.

The crystallization (solidification) of pure elementary metals, such as aluminum and copper, occurs at a single sharply defined temperature level, known as the freezing point. The transition from the liquid to solid states of all initial compounds, including steel, which is an alloy, takes place over a temperature range, the limits of which depend on the specific chemical composition of the compound. On cooling from the liquid or molten state, a mild steel begins to solidify upon reaching the "liquidus" temperature and the solidification is completed on reaching the "solidus" temperature. In the zone between the liquidus and the solidus temperatures, the alloy consists of two phases: solid solution

2

delta and of liquid iron. In this state, the alloy has little or no cohesive strength, and is generally referred to as being in the "mushy" range.

The higher liquidus temperature and considerably lower thermal conductivity of steels in comparison to the freezing point of copper and aluminum affect the casting process. For example, the liquidus temperature of most steels is of the order of 750 F. higher than the freezing point of copper, and 1500 F. higher than that of aluminum. The thermal conductance of most steels is of the order of from 3-12% that of copper, and from 6-23% that of aluminum.

The higher temperature of crystallization and heat content of steel, when in the molten state, necessitates a much greater rate of heat abstraction from the heat receiving surface of the mold wall in order to maintain the receiving surface temperature at a temperature which will not cause adhesion of the metal being cast to the mold. Furthermore, with the lower thermal conductivity of the steel a wide temperature difference will exist between the surface and the interior of a body of steel being cast dependent upon the rate of heat removal from the surface of the body of steel.

The continuous casting of copper and aluminum does not involve any substantial slag removal problem, whereas the removal of slag presents a major problem in the continuous casting of steel. In the melting of copper and aluminum, the erosive characteristics of the slag and the comparatively low temperatures involved have only a moderate disintegrating effect on the refractories lining the furnace or other receptacles in which these materials are melted or handled. These conditions are much more severe in the manufacture of steel where the development of a slag is a prerequisite for the purification of the metal and also in view of the fact that the non-metallics and iron compounds attack most refractories commonly used for lining receptacles in which steel is handled.

A better understanding of the present invention can be gained from a consideration of the specific problems encountered in the continuous casting of steel. These problems may be divided into two general, but inter-related, subdivisions, i. e., the physical problem of continuously casting steel and the metallurgical problem of obtaining a commercially acceptable semi-finished or finished steel product from such a continuous casting process.

Referring to the physical aspects of the problem, the basic apparatus for the continuous cast-

ing of metals includes a fluid cooled mold, open at both ends, which is arranged for the introduction of molten metal into the upper end thereof and the withdrawal of the casting from the lower end of the mold. One of the primary problems of continuous casting is the provision of an adequate cooling effect on the mold wall to solidify the metal within the mold. This is primarily a heat transfer problem.

One of the principal difficulties encountered in the continuous casting of steel lies in the tendency of the solidified metal to stick to the wall of the mold. This is believed to be the result of improper cooling due to one or more of several factors, such as improper mold material and thickness, inadequate cooling fluid conditions, oxidizing atmosphere at the molten metal level, the presence of slag in the metal, and rate of casting withdrawal. Sticking to the mold tends to cause rupture of the initially formed thin walled embryo casting.

If the poured metal is too cold or if the mold cooling is too rapid, then shrinkage of the embryo casting from the mold wall takes place rapidly enough to permit additional metal to flow over the frozen rim of the casting and thus cause possible jamming of the casting in the mold with a subsequent break at the point where the casting shell reheats from the flow of heat from the semi-molten and molten central portion of the casting. If a rupture occurs within the mold, the uppermost section of the embryo casting adheres to the mold while the lower section continues to be withdrawn. Generally, the uppermost section will not free itself sufficiently by shrinkage to permit its withdrawal by the embryo shell formed by the metal that has flowed outwardly from the center to fill the ruptured gap unless a momentary stoppage is created thus allowing the shell to thicken and subsequently free itself by shrinking in the normal manner. In the event that the operation is not stopped when the "sticker" occurs, it is likely that the shell formed by the metal that has filled the rupture will be too thin to stand the downward pull of the previously solidified casting and repeated ruptures will take place, until finally a rupture occurs at the bottom end of the mold where the metal is free to run from the casting, thus leaving an empty shell of solidified metal clinging to the interior of the mold.

It is imperative that the ferrostatic head of molten metal be maintained on the embryo casting and as long as this head is maintained an off-center delivery of molten metal to the mold will have no appreciable effect on solidification. The problem of casting is dynamic, with the variables being the rate of withdrawal, rate of pour, degree of metal superheat, and rate of heat transfer from the solidifying metal. The metal will draw away from the mold wall only after initial solidification and formation of the shell. Since this condition is dynamic, it is only harmful when the rate of casting withdrawal is too slow for the rate of solidification and new metal entering the mold flows down between the shell of the embryo casting and the mold wall, wedging the casting to the mold. The superheat temperature of the molten metal as poured and rate of withdrawal of the casting primarily affect the length of the molten core and the porosity of the solidified casting rather than the formation of the shell.

To justify economically the capital investment for a continuous casting apparatus, it is neces-

sary to attain a relatively high casting rate. This requires a high rate of heat absorption from the molten metal in the casting mold. A high rate of heat absorption from the molten metal within the casting mold and the comparatively low thermal conductivity of ferrous metal combine to permit a quick formation of a solidified shell for the embryo casting. As the shell thickens, the solidified metal tends to shrink away from the mold wall. The shrinkage of metal from the mold wall reduces the friction therebetween, which is of advantage from the standpoint of some of the physical problems of continuous casting. However, shrinkage of the metal also introduces a heat exchange problem due to the change in heat transfer characteristics between a condition involving heat conduction from the molten metal to the contacting mold wall, and heat transfer across the gap between the surface of the embryo casting and the mold wall.

The low thermal conductivity of steel and the mushy transition stage through which it passes result in the formation of an elongated V-shaped molten core surrounded by a similarly elongated V-shaped mushy core in the casting which introduce serious metallurgical problems in the continuous casting of ferrous alloys. Also, due to the time-temperature relationship in the formation of the embryo casting, a rapid cooling to form the skin, followed by further rapid cooling to solidify the core, will invariably result in thermal stress cracks, cores, porosity and/or dendritic cracks within the casting. Porosity in the steel casting, exclusive of porosity caused by gas inclusions, is primarily due to the change in specific volume which takes place in the solidification of the molten metal. This is a purely physical characteristic and when porosity occurs in the finished casting it can be attributed to a lack of molten metal feed to the embryo casting to fill the voids formed during the solidification of the metal. Such conditions within the cast product are naturally undesirable and may be alleviated or eliminated by varying casting temperature, rate of pour and rate of heat removal, the latter operation being important both in the mold and after the ingot has been withdrawn therefrom. There is a very complex balance between these variables.

Any slag and impurities carried down into the mold tend to collect on the periphery of the embryo casting. Since slag has a lower heat conductance than steel, any slag trapped in or on the thin shell of the embryo casting will tend to insulate the covered portion of the casting from the heat removal effect of the mold wall, so that the shell strength of the casting may be insufficient to withstand the ferrostatic pressure imposed thereon, and may result in a rupture of the shell. It has also been observed that where the solidification of the adjacent interior portion is delayed, its subsequent solidification and shrinking sometimes results in the formation of shrinkage cracks and voids in that area.

The principal object of the present invention is to provide a process of and an apparatus for the continuous casting of metal in semi-finished or finished products of a commercially uniform and acceptable quality at a commercially economical rate of production. A further and more specific object is to provide a method and apparatus of the character described capable of effecting the production of semi-finished or finished ferrous and other high melting point alloy products of indeterminate length which is characterized by

a longitudinal uniformity of metal density and structure. An additional specific object is to provide a process and apparatus of the character described for continuously receiving molten metal poured into one end of an open-ended liquid cooled mold, chilling the molten metal within the mold at a rate of heat transfer sufficient to form an embryo casting, and continuously withdrawing the embryo casting from the opposite open end of the mold with the embryo casting having sufficient strength to withstand the ferrostatic pressure of its molten and mushy interior without rupture or distortion. A further object is to provide a method and apparatus for the continuous casting of ferrous and other high melting point alloys wherein the temperature of the molten metal delivered to an open-ended, liquid-cooled mold is maintained at a substantially uniform temperature. An additional object is to provide a method and apparatus of the character described wherein the composition of the metal, the rate of molten metal delivery to the mold, the cooling rate of the metal within the mold, and the rate of withdrawal of the casting from the mold are co-ordinated to establish and maintain the production of a substantially uniform high quality casting at a commercially economical rate. A further object is to provide a method and apparatus of the character described in which the casting is subjected to a delayed cooling, soaking or reheating zone to solidify the metal in the casting while maintaining a substantially uniform and minimum temperature gradient transversely of the continuous casting, whereby the structure of the cast product will be substantially uniform throughout its length.

In accordance with the process of the present invention, we are able to continuously cast various ferrous and other high melting point alloy products, each of commercially acceptable quality and of a substantially uniform metallurgical structure throughout its indeterminate length. In the continuous casting of steel, for example, steel of the desired composition is first melted in accordance with good steel making practice and delivered to a suitable holding and/or pouring ladle. The ladle may be advantageously constructed with metal heating means, operable in case of delay in pouring the molten metal, to insure that at the time of pouring, the metal temperature will be within an optimum temperature range, which, while varying with the metal composition, will normally be about 150-200° F. above the liquidus temperature of the metal. As much as possible of the slag present in the charge is removed from or retained in the ladle. The molten metal is poured at a controlled rate into a tun dish constructed to substantially eliminate the velocity head of the poured metal, retain the remaining slag in the tun dish, and deliver the clean molten metal at a substantially uniform temperature and low velocity head centrally of a continuous casting mold.

To minimize the amount of slag in the charge, the refractory linings of the parts in contact with the molten metal are constructed of the same ceramic composition. For example, when the metal is melted in an electric arc furnace lined with a magnesium oxide refractory, as is the customary practice, all the refractory linings thereafter in contact with the molten metal, i. e. the linings for the ladle or ladles and tun dish, should likewise be made of similar magnesium oxide refractories. The use of similar or compatible refractories tends to avoid chemical re-

actions between the slag formed by the reaction of molten metal with one type of refractory lining, with a lining of another refractory composition.

5 A special stationary casting mold assembly is employed which is constructed and operable to permit the desired high rate of heat absorption from the molten metal and embryo casting formed to be maintained. The casting mold itself is 10 upright and open at both ends, and the delivery rate of molten metal to its upper end is coordinated with the rate of withdrawal of the casting from its lower end to maintain in normal operation a reasonably uniform level of molten metal within and below the upper end of the mold. The liquid level should not be carried too close to the top of the mold because of both 15 atmospheric and cooling fluid conditions. A substantially uniform ferrostatic head of molten metal is thus maintained on the shell of the embryo casting so as to obviate rupture of the shell. The stream of molten metal delivered is also regulated by adjusting the position of the tun dish, to enter the molten pool along the axial 20 center-line of the mold with a minimum of splashing against the mold and so as to avoid turbulence in the molten metal pool in the mold. A quiet pool of metal has been found to promote 25 uniform circumferential cooling in forming the solidified shell of the embryo casting.

30 The maintenance of a negative meniscus on the upper surface of the molten metal in the mold has been found to be important, if not an essential condition, to successful operation. The character of meniscus formed by the molten metal will depend upon whether a wetting or non-wetting contact exists between the molten metal and the adjacent mold surface. We have observed that the presence of oxides, principally iron oxide, 35 and other impurities on the molten metal surface tends to cause wetting of the adjacent mold surface and thus lead to sticking of the casting in the mold, as is evidenced by the formation of a positive meniscus on the molten metal. We have found that complete elimination of oxygen from the mold atmosphere above the molten metal is highly desirable to prevent formation of such oxides. This is accomplished by the continuous 40 introduction of an inert gas, preferably heavier than air and non-soluble in the metal, into the top of the mold to displace any lighter gas, such as air, therefrom and also the introduction of a substance which will consume any oxygen and/or reactive gases that might remain in the mold. The combined effect produces a substantially oxygen-free atmosphere in the mold space immediately above the molten metal level.

45 Our process of continuous casting of ferrous and other high melting point alloys is particularly distinguished by the extremely high rate of mold cooling employed. While the prior art has appreciated that the casting of ferrous alloys would require a somewhat higher mold cooling rate than the casting of copper and aluminum, for example, we have found by extensive experimentation that a ferrous alloy casting cannot be successfully made at an economical casting rate and with commercially acceptable quality, with a rate of heat transfer from the portions of the mold effective in the formation of the embryo casting which is less than several times over the maximum cooling rate heretofore recommended by the prior art for ferrous alloys. This extremely high cooling rate is attained in our process by the introduction of the cooling liquid into

the mold assembly in a manner and in quantities insuring the entry and maintenance of a solid stream of cooling liquid throughout the mold cooling passage to eliminate cavitation effects, the flow of cooling liquid through the passage at a velocity having a calculated Reynolds number for highly turbulent flow conditions, a temperature gradient from the molten metal to the cooling liquid such as to minimize the temperature difference between the liquid-contacting liner surface and the cooling liquid, and also a minimum temperature rise in the cooling liquid itself between its points of entry and discharge from the mold passage.

We obtain a metallurgically sound continuous casting by the co-ordination of the described rapid chill to form a shell or skin for the casting of adequate strength to avoid run outs by the interior molten metal, followed by a controlled cooling, or in some cases by externally reheating the casting, after it leaves the mold. The best and most uniform grain structure in a sound steel casting is obtained by maintaining a minimum temperature gradient between the center of the casting and its periphery throughout its remaining period of solidification. Such conditions require a time and temperature control of the cast product that are entirely different from conditions in a conventional steel casting operation. In the delayed cooling or reheating zone the solidified shell is reheated by externally supplied heat or by heat exchange with the hotter core. As a result, the temperature gradient from the center to the periphery of the cast product will be minimized and, as the molten and mushy core gives up its heat of fusion to the solidified skin, the casting will become solidified throughout. During this controlled solidification of the casting, any voids therein created by metal shrinkage will advantageously be afforded sufficient time to be filled by molten metal from the upwardly adjacent molten metal core. Due to this slow and controlled cooling, the core of the casting is of appreciable length and thus acts in somewhat the same fashion as the hot top ordinarily used in the steel industry, tending to avoid internal and external stress cracks in the finished casting.

The descending continuous casting, when below a point where solidification is complete, is periodically cut into a predetermined length by suitable metal cutting mechanism, for subsequent ease of handling and delivery to the point of use.

The various features of novelty which characterize our invention are pointed out with particularity in the claims annexed to and forming a part of this specification. For a better understanding of the invention, its operating advantages and specific objects attained by its use, reference should be had to the accompanying drawings and descriptive matter in which we have illustrated and described a preferred embodiment of our invention.

Of the drawings:

Fig. 1 is an elevation view of a continuous casting apparatus constructed in accordance with the present invention;

Fig. 2 is an enlarged side view, partly in section, of a portion of the apparatus shown in Fig. 1;

Fig. 3 is an end view taken on the line 3—3 of Fig. 2;

Fig. 4 is an enlarged view of a portion of the apparatus shown in Fig. 3;

Fig. 5 is a side elevation, partly in section, of the tun dish assembly as viewed from line 5—5 of Fig. 8;

Fig. 6 is a cross-section view of the tun dish; Fig. 7 is a plan view of the tun dish assembly; Fig. 8 is a front elevation view of the tun dish assembly with certain portions thereof broken away to show details of construction;

Fig. 9 is a section taken on line 9—9 of Fig. 8; Fig. 10 is an enlarged sectional elevation of another portion of the apparatus shown in Fig. 1;

Fig. 11 is a further enlarged sectional elevation of part of the apparatus shown in Fig. 10;

Fig. 12 is a plan view of the apparatus shown in Fig. 10;

Fig. 13 is an enlarged plan view, partly in section, of the casting cutting apparatus;

Fig. 14 is a vertical section taken on the line 14—14 of Fig. 13;

Fig. 15 is a horizontal section taken on the line 15—15 of Fig. 14;

Fig. 16 is an enlarged elevation of the severed casting handling apparatus shown in Fig. 1;

Fig. 17 is an elevation of the dummy rod used in the continuous casting operation;

Figs. 18 and 19 are operations charts of typical casting runs with the apparatus shown in Figs. 1—17.

While various features of our improved process and apparatus are adapted for use in the continuous casting of both low and high melting point metals and alloys, our process and apparatus described herein are particularly designed and especially useful for the continuous casting of carbon and alloy steels as well as nickel and high melting point alloys.

In the continuous casting apparatus shown in the drawings, molten steel or other ferrous metal or alloy is introduced at one end of the apparatus and semi-finished products ready for final shaping and finishing are delivered from the opposite end. The assembly of the apparatus is shown generally in Fig. 1, while the details of the parts are shown in Figs. 2—17. As shown in Fig. 1, molten steel is transported to the apparatus by a transfer ladle 10 from a melting furnace (not shown) and bottom poured to a suitable holding and pouring ladle 11 which is constructed and operated to maintain the molten metal therein at a selected temperature, in this case by induction heating. The ladle 11 is arranged for lip pouring with a regulating mechanism designed to effect a continuous selected pour rate into an adjustably positioned tun dish 12 which discharges the molten metal into the upper end of and along the axial center of an associated casting mold assembly 12. The molten metal is rapidly chilled in the mold assembly 12 to form the shell or skin of an embryo casting and solidification of the casting completed in a subsequent delayed cooling or soaking section 63, the casting being continuously withdrawn therefrom as a continuous casting 13 at a controlled rate by a set of power-driven pinch and/or withdrawal rolls 14, with the continuous casting thereafter passing to the handling portion 15 of the apparatus where the casting 13 is cut into predetermined lengths and each length as cut delivered to a horizontal conveyor for transportation to a point of use or storage (not shown).

The pouring ladle 11 and its operating mechanism shown in Figs. 2, 3 and 4 is disclosed and claimed in a co-pending application of I. Harter, Jr. and S. O. Evans, Serial No. 746,810 filed May 8, 1947, now Patent No. 2,520,598, issued August

29, 1950, and comprises a lining of refractory blocks 16 and plastic refractory 17 for a water-cooled induction coil 20. The coil 20 is supported in a box 21 of a cemented asbestos material 22. The ladle bottom and removable top 23 are also lined with suitable refractory materials. The ladle 11 has a pouring lip 24 in its side wall adjacent the upper end of the coil 20. In order to control accurately the delivery point of the stream of molten metal into the tun dish 18 from the lip 24 of the ladle, the ladle is tiltable about a horizontal axis X—X laterally of and movable relative to the mold assembly 12. The ladle is mounted on an L-shaped frame 25 having trunnions 26 engaging trunnion bearings 27 on pedestals 30. As shown in Fig. 3, the lower edge of the lip 24 preferably lies on the axis X—X. The trunnion bearings 27 are slideable horizontally on guides 31 on the pedestals 30, the lateral position of both bearings being simultaneously regulated by screws 32 operated by a pair of interlocked reversing type gear motors (not shown). The tilting movement of the frame and ladle is effected through a cable 33 attached to a cable yoke 34 on the frame 25. The cable 33 is passed through a pair of conventional differential chain blocks 35 and is wrapped about a grooved drum 36 rotated by a reversible motor driven gear drive. The uppermost block 35 is supported from the supporting framework for the drum 36 and its drive, so that the frame and ladle can be rotated through an angle of approximately 90° about the axis X—X.

The electrical and cooling water connections to the ladle coil 20 are flexible to permit rotation of the ladle about axis X—X. The flexible electric cables 40 are alternately attached to water-cooled pipes 41 leading to the coil 20 to minimize electrical loss and reactance. From the pipes 41 the cables 40 pass over a grooved drum 42 mounted in the frame 25, and over a grooved drum 43 on the building frame-work. The cables 40 are then looped downwardly around a grooved drum 44 which acts as a counterweight to maintain proper cable alignment. The cables 40 lead to the electrical control and frequency generating equipment located at a lower level and indicated generally at 45 in Fig. 1. The flexible water connections to the pipes 41 are arranged so that tilting of the ladle will not interfere with the flow of cooling water to the coil.

Thus by regulation of the horizontal position of the trunnion axis X—X relative to the mold 12 and the angularity of the ladle longitudinal axis relative to the vertical, the pouring rate of metal from the ladle can be regulated and the point of delivery of that metal to the tun dish 18 can be controlled. Likewise, the temperature of the metal within the ladle and therefore the temperature of the metal delivered to the mold, can be readily maintained within optimum limits for most advantageous casting results. The three variables commonly present in the delivery of molten metal to a continuous casting mold, namely, metal temperature, pour rate, and position of metal delivery into the tun dish should be maintained within optimum limits such as, for example, by the described construction of the ladle 11. The control of these variables is highly important in the operation of a successful commercial continuous casting operation, particularly in the casting of ferrous and other high melting point alloys.

The tun dish 18 and supporting provisions shown in Figs. 5 to 9, are disclosed and claimed in a co-pending application of T. W. Ratcliffe et

al., Serial No. 2,114, filed Jan. 13, 1948, now Patent No. 2,571,033, issued October 9, 1951, the tun dish being adjustable to receive molten metal from the ladle 11 and to deliver that metal in a continuous stream to the axial center of the mold assembly 12 at the normal molten metal level therein. In order to absorb the impact of the falling stream from the ladle and to return any entrapped slag to the surface and at the same time constrain and direct the turbulence caused by the falling stream, the tun dish consists of an open top refractory lined rectangular box divided into an inlet chamber 18<sup>a</sup> and a smaller outlet chamber 18<sup>b</sup> by a transverse vertical refractory baffle or partition 19 located approximately one-third of the length from the discharge end. A transverse inclined refractory baffle section 19<sup>a</sup> is located in the inlet chamber and extends upwards at an angle of approximately 20°-30°, with its lower and forward end merging into the vertical baffle 19. Holes 28 in the bottom of the vertical baffle below its juncture with the inclined baffle form separate passages through which the molten metal can flow from the inlet to the outlet chamber. A V-notch refractory weir 29 is formed in the end wall of the tun dish for the discharge of the molten metal. In operation, the tun dish is preheated to a high temperature and normally tilted forwardly about 15° and the tun dish positioned so that the stream of molten metal from the ladle 11 falls into the inlet chamber and strikes the vertical baffle 19 below the normal molten metal level in the chamber at such an angle that the stream continues to descend until it strikes the inclined baffle 19<sup>a</sup>, which deflects the metal-entrapped slag to the surface, from which it can be removed. The slag-free metal then flows over the inclined baffle and downwardly through the passages 28 in the vertical baffle to the outlet chamber 18<sup>b</sup>, from which it flows approximately horizontally through the V-notch weir 29.

The tun dish is removably mounted in open trunnion bearings 37 adjustably supported on a horizontally swinging arm 38 which permits the tun dish to be swung away from the vicinity of the mold for ease in handling. While the tun dish is on the arm and in operation it can be tilted in a vertical plane about an axis located in line with the crest of the weir 29, turned in a horizontal plane about a point directly under the weir, and moved horizontally along its short axis. These motions are primarily for the purpose of correcting any misalignment of the metal stream which may be caused by frozen slag or metal on the weir and thus enable the operator to more accurately direct the stream into the center of the molten pool in the mold. The tilting of the tun dish is effected by a screw crank 49 contacting with a depending arm 49<sup>a</sup> secured on one of the tun dish trunnions. Angular movement of the tun dish about a vertical axis is effected by mounting the tun dish trunnion bearings 37 on a separate plate 58 having a pivotal connection 58<sup>a</sup> with an extensible section 38<sup>a</sup> of the arm 38 and a screw crank 58<sup>b</sup> removably mounted on the outer end of the plate engaging a pivoted nut 58<sup>c</sup> on the extensible arm section 38<sup>a</sup>, so that operation of the crank will cause the plate 58 to move angularly about the vertical axis of the pivotal connection 58<sup>a</sup>. Lateral movement of the tun dish is effected by an arcuate slide 59 engaging a fixed arcuate flange 58<sup>d</sup> on the

opposite end of the plate 58. The slide 59 carries a laterally projecting bolt 59<sup>a</sup> on which is threaded a turn nut 59<sup>b</sup> carrying a bevel gear 59<sup>c</sup> at its outer end. A bevel gear 68 carried by a crank 68<sup>a</sup> on the arm 38 engages the gear 59<sup>c</sup> to cause the bolt 59<sup>a</sup> to move laterally and adjust the position of the arm section 38<sup>a</sup> and plate 58. The pivotal connection 58<sup>a</sup> is constructed to permit such lateral movement relative to the arm 38.

In operation the tun dish thus serves as a slag barrier which tends to prevent the inclusion of extraneous matter in the metal delivered to the mold. Although the molten metal delivered to the ladle 11 is essentially "clean," any induction heating therein tends to agitate the metal and frequently metallic oxides or other impurities will accumulate on the surface of the metal which are advantageously caught and removed in the tun dish before delivery to the mold assembly 12. As shown in Figs. 2 and 5, the tun dish weir 29 is close to the mold assembly to minimize oxidation of the discharging molten metal and turbulence of the molten metal in the mold.

The desired extremely high rate of mold cooling employed is obtained by utilization of the fact that the rate of heat transfer from the mold wall will vary as a direct function of the velocity of the cooling liquid, provided no cavitation effect or laminar flow is present in the cooling liquid passage. The mold assembly 12 for this purpose, shown in detail in Figs. 10, 11 and 12, is arranged to remove heat from the molten metal delivered to its upper end, and to continuously develop an embryo casting therein which is continuously withdrawn from its lower end as hereinafter described. While in the mold assembly, the molten metal and the embryo casting are in contact with or adjacent to the inner surface of a water cooled vertically elongated relatively thin walled metallic molding tube or mold liner 46 which is open at its upper and lower ends and of the desired casting cross-section, in the present embodiment one of circular horizontal cross-section. The upper open end of the tube is supported in a top plate 47, whereby the tube is pendentally supported from the fixed level of the plate and is free to expand axially therefrom. The plate 47, forms the top wall of an annular chamber 56, defined by a cylinder 54 mounted on a load carrying bottom plate 55, which rests on structural supports (not shown).

A metallic tubular member or skirt 52 of corresponding cross-sectional shape surrounds the mold liner 46 and is arranged to confine a flow of cooling liquid against the surface of the mold liner substantially throughout its length. The skirt is also pendentally supported adjacent its upper end by attachment within the central aperture of the plate 55. The upper end portion of the skirt 52 extends above the level of the support plate 55, with its upper edge fitting into a corresponding recess in a surrounding sleeve 60, secured on the upper side of plate 55, and defining a discharge weir from the chamber 56. A relatively narrow annular open-ended space or water passage 53 of uniform width is thus provided between the liner 46 and skirt 52.

A plurality of cooling water inlets 57 open to the chamber 56 at uniform circumferentially spaced positions, and an annular perforated distribution plate 61 is interposed between the inlets and the water passage 53. The upper end or weir

section of the sleeve 60 is shaped to form an anti-cavitation entrance nozzle to the water passage 53, the upper end of the sleeve being rounded and its inner wall cut away to converge at an angle  $\alpha$  of approximately 20° to a diameter corresponding to the inner diameter of the skirt 52.

The lower end of the skirt 52 is spaced from the lower end of the liner 46, both the liner and the skirt being unrestrained relative to one another at positions below plate 55, so that each may adjust itself in accordance with the temperature and loading imposed by the enclosed metal or the cooling liquid. The length of the mold liner 46 will depend upon various factors, such as the composition of the metal, casting cross-section and the desired rate of withdrawal of the casting. The mold liner illustrated when used for casting 6" rounds was made 108" long. In such a mold assembly the radial thickness of the water passage 53 is approximately  $\frac{1}{8}$  inch. As high rates of heat transfer from the cast metal to the water are involved, the wall thickness of the mold liner 46 is advantageously low and where the liner has been made of brass a thickness of  $\frac{1}{4}$  inch has been utilized. Where the mold liner is made of other material, such as mild steel, stainless steel or copper, consideration of the somewhat different heat conductivity characteristics will of course be involved in the determination of the related dimensions of the heat conductive mold liner.

The location of the converging entrance between the upper end of sleeve 60 and the outside of the liner 46 so as to receive a cooling water supply from the upper annular portion of the chamber 56 above the perforated plate 61, insures a uniform solid stream of water into the passage 53 throughout its circumference. In addition, the gradually converging entrance also provides for a gradual acceleration of the water velocity to a rate, at the entrance of the annular water passage 53, which will be well within the range of turbulent flow conditions, thus insuring a high rate of heat transfer from the outer wall face of the liner 46 to the cooling water. In attaining this condition, relative outside and inside diameters of the liner 46 and the skirt 52 are so selected that, with the rate of circulation and temperature of the water discharged therethrough, a calculated Reynolds number will result which will insure highly turbulent flow conditions through the passage.

The lower end of the mold liner 46 is provided with a frusto-conical water deflecting shield 50 below the skirt 52 and which is arranged to deflect cooling water away from the embryo casting as it emerges from an annular opening 73 at the lower end of the liner 46. The arrangement of the parts described cooperate to form a water-cooled portion of the mold assembly 12 wherein a high rate of heat exchange between the molten metal introduced into the top and the cooling water flowing on the outside of the liner 46 can be maintained to solidify an outer skin on the embryo casting which will thicken as the casting is withdrawn downwardly as hereinafter described.

In initiating the operation of the continuous casting apparatus, a dummy 164, such as illustrated in Fig. 17, is inserted in the mold with its upper end positioned intermediate the length of the mold liner 46 and with its lower end engaged by the pinch rolls 14. The dummy 164 is constructed in a series of short sections 165 for convenience in handling, with adjacent sections held

together by means of pins 166 so that the dummy may be readily assembled and disassembled.

After molten metal has been delivered to the pouring ladle 11 and the metal has been heated to the desired pouring temperature therein, cooling water is circulated through the mold 12 and molten metal is delivered to the mold cavity formed in the liner 46 by the dummy 164. When the molten metal level in the mold liner 46 has reached a predetermined point adjacent its upper end, the pinch rolls 14 are started to withdraw the dummy 164 at a uniform selected rate co-ordinated with the casting variables to form a metallurgically sound casting. The dummy extends from the rolls 14 to an intermediate position within the mold liner 46, and as each successive section 165 of the dummy projects below the rolls 14, the pin 166 is withdrawn and the section removed for future use. A head 167 on the upper end of the dummy 164 is provided with a cap screw 168 threaded into the upper end thereof. The lower end of the continuous casting 13 solidifies around and grips the upwardly extending shank and head of the cap screw 168, whereby the initially formed casting 13 can be withdrawn from the mold by the pinch rolls 14 acting on the dummy 164.

Liquid or gaseous materials are introduced into the upper portion of the mold, above the level of molten metal therein, to provide a non-oxidizing atmosphere above the molten metal. Such liquid materials are largely gassified by the high temperature conditions within the mold, and the primary effect on the gas will be to provide a non-oxidizing atmosphere for the molten metal in the upper end of the mold. Tubes for introducing liquid and gaseous materials into the mold are shown in Figs. 10, 11 and 12 as arranged in circumferentially spaced pairs about the upper end of the mold assembly 12. One tube 77a in each pair is connected with a positive displacement flow control mechanism (not shown) whereby a liquid, such as castor oil, may be delivered to the mold, while the other tube 77b is connected with a source of an inert gas (not shown), such as argon. Argon, being heavier than air will collect in the upper end of the mold above the surface of the molten metal therein, so that oxygen-containing, reactive or metal soluble gases will be displaced and the molten metal pool and the entering stream of metal will be protected against oxidization thereof. The exact function of the castor oil in the continuous casting process is not completely understood. Its use seems to be advantageous under some casting conditions, particularly during the initial casting period. By observation, it is believed that the castor oil is vaporized after entering the mold and at least partially decomposed in the vicinity of the meniscus of the metal within the mold. The hydrogen released in the decomposition of the castor oil vapor tends to combine with any oxygen present, thereby reducing any tendency for the formation of metallic oxides by oxygen contact with the molten metal. The quantity of castor oil introduced through each of the tubes 77b amounts to only one to four drops per minute, which is equivalent to approximately .05 to .20 pound per ton of metal.

In the operation of the molding apparatus, cooling water, with or without the addition of a suitable "wetting agent", is introduced to the upper end of the mold 12 through the pipe connections 57. With the described construction

of the entrance section of the passage 53, the water entering the chamber 56 will flow downwardly through the annular passageway 53 in a uniform solid stream. In order to obtain the necessary rate of heat transfer to successfully continuously cast ferrous alloys at commercial lineal speeds, it is believed to be essential that a large amount of cooling water be passed through the annular passageway 53. The amount will vary with the casting cross-sectional area and shape and the speed of withdrawal maintained, but in general should be such that the average rise in cooling water temperatures through the mold assembly will be less than 12° F. The maximum cooling rate we have noted in the prior art for ferrous alloys is 30-35 gallons per minute at a head pressure of 75-150 p. s. i. for 6" steel rounds (Patent No. 2,079,644). We have found it advantageous, if not essential, to use a cooling water flow of 350-400 gallons per minute at an entering water main temperature and a head pressure of 75-100 p. s. i. for continuously casting 6" steel rounds in a mold assembly similar to that illustrated herein. With such cooling water flow rates through the water passage 53, the water velocity therein will be from 43-50 feet per second. Thus, allowing for the usual manufacturing tolerances for the dimensions of the mold liner and skirt, the water flow velocity should be at least 40 feet per second. Consequently it is an essential part of our ferrous alloy casting process that the amount of cooling water supplied should be at least several times over the maximum amount heretofore recommended by the prior art for such casting. A high ratio of cooling water supplied relative to pounds of metal cast per minute thus results. We have found that at low flows of cooling water a falling stream can burn through the side of the mold when the stream becomes deflected while entering the mold cavity.

Due to the relatively restricted cross-sectional area of the flow passage 53, the water flow therethrough will be at a high velocity for effective heat transfer thereto from the outer surface of the mold liner 46. For most effective heat transmission between the mold liner and the cooling water the water flow through the passage 53 should be maintained at a velocity having a calculated Reynolds number indicating a highly turbulent flow rather than a laminar flow. Since the annular discharge end of this water passage is unrestricted and the water discharges into an annular area at atmospheric pressure, the pressure of the cooling water is converted substantially from a static pressure to a velocity pressure. The continuity, velocity and direction of the water stream is thus maintained throughout the length and periphery of the passage. This pressure conversion avoids any tendency for the high static pressure of the water to distort the mold liner 46, which would result in an uneven circumferential cooling of the casting within the mold. Any distortion of the mold liner by reason of expansion and contraction with temperature change would have a further destructive effect upon the formation of the casting in that the casting might have a tendency to bind in the mold and with such an interruption in withdrawal continuity the fragile skin of the embryo casting is apt to rupture. Distortion and/or buckling of the mold is avoided in the construction shown since the component parts are free to expand axially of the mold,

Below the lower end of the skirt 52 and shield 50 is a delayed cooling or reheating zone, or temperature equalizing section, 63, defined by a pair of spaced concentric cylindrical sleeves 64 and 65 which are coaxial with respect to and spaced from the embryo casting formed in the upwardly adjacent mold. The sleeves are constructed in a variable number of longitudinal sections and the annular space between the sleeves is filled with a temperature resistant heat insulating material 66 maintained in position by upper and lower annular plates 67 and 70 respectively. Cooling water discharging through the annular opening 73 is deflected outwardly by the shield 50 and a frusto-conical plate 71 to pass downwardly between the outer sleeve 65 and a cylindrical sleeve 74 into a reservoir or tank 75. The tank 75 is annular in horizontal cross-section and is provided with a cylindrical inner wall 75a coaxial with the casting and of the same internal diameter as that of the sleeve 64. Thus the casting formed in the mold continues to be cooled, but at a substantially reduced rate and without direct contact with any cooling water.

When the continuous casting process has been started, with the rate of molten metal delivery to the mold coordinated with the predetermined rate of withdrawal of the casting, thus maintaining a substantially uniform ferrostatic pressure on the casting, the liquid metal will start to solidify in a boundary layer or skin along the internal wall of the mold liner 46. In the apparatus shown and with the desired rate of supply of cooling water introduced through the connections 57, the skin will start to form within a fraction of an inch of the meniscus of the molten metal and since the distribution of cooling water is substantially equal circumferentially of the mold, the skin formation will also be substantially uniform throughout its circumference. Almost immediately the solidified skin on the casting will shrink away from the mold wall with an attendant reduction in heat transfer by conduction to the mold wall. We believe that the shrinkage gap between the casting and the wall will gradually increase with an increase in skin thickness until the total heat transfer to the mold liner, by both conduction and radiation, is finally overcome by the heat flow from the molten core of the casting to the skin. When this unbalance of heat transfer occurs the thickness of the skin will gradually be reduced with the inner surface of the solidified metal reaching a mushy or plastic stage. As the casting is drawn further down through the mold the gradual reheating of the skin from the molten core will be reduced to a point where the heat removal from the skin to the mold will again be the greater and the skin thickness will again gradually increase.

It is also our belief that at the instant of initial crystallization a fine-grain shell forms because it is essentially chill cast. Immediately long thin dendrites form increasing in thickness and length as the temperature of the molten core decreases. If the dendrites do not reach the geometric center of the section by the time the core temperature reaches the solidus, nucleation will increase rapidly and the balance of the molten mass will freeze at one time causing a central pattern of equiaxial crystals. The temperature gradient from the central core to the outer surface may and can cause solid transformations such as occur in the transition of martensite to bainite. in

an incomplete water quench of a medium to high carbon steel. There is a range of casting thickness when the cooling rate must be lowered in order to obtain a sound ingot. Our experience has shown that it is advisable to avoid the formation of large quantities of equi-axed crystals.

Ordinarily, the casting variables, such as the metal level in the mold, metal pouring temperature and the mold cooling rate are maintained in a substantially balanced or coordinated condition during the casting process. Any minor change in the casting variables usually occurs in the rate of molten metal delivery to the mold and can be corrected by a corresponding compensation in the rate of casting withdrawal from the mold. A more drastic change in one or more of the casting variables may result in a "sticker," necessitating a momentary stoppage of the casting withdrawal mechanism which is immediately followed by a resumption of the casting withdrawal. Such an interruption in the continuity should, of course, be avoided for high quality casting production, but is relatively harmless to the process.

Our understanding of the formation of the embryo casting is shown in Figs. 10 and 11 wherein the thickness of solidified metal forming the skin 80, the mushy metal 81 and the molten core 82 of the casting are exaggerated for illustrative purposes. The "air" gap 83 between the mold liner 46 and the skin 80 is shown in exaggerated dimensions in Fig. 11, while due to the small scale of Fig. 10 the "air" gap 83 is not illustrated. In Fig. 10 we have illustrated the formation of a continuous casting within the mold as heretofore described. It is, of course, understood that the distances between the various zones shown will vary with the type of metal cast, the rate of casting withdrawal, and the rate of cooling; however for the production of most low carbon steels, the illustration is considered approximately correct. At the level A the metal adjacent the mold liner 46 becomes mushy or plastic with its thickness gradually increasing to the level B where a frozen metal shell or skin 80 starts to form. Between the levels B and C the thickness of both the mushy metal 81 and the skin 80 gradually increases, while between levels C and D the skin 80 gets thicker and then thinner as heretofore described. Between the levels D and E, the thickness of the skin 80 gradually increases until at level E the molten core 82 disappears. Between the levels E and F the area of mushy metal 81 is gradually reduced to the level F where the casting is completely solidified.

The removal of heat from the molten metal in the upper part of the mold liner 46 is accomplished primarily by conduction due to the direct contact of the metal with the inner surface of the mold liner. This heat transfer rate is extremely high. As the metal contacting with the mold liner solidifies to form the skin 80 of the embryo casting, the outer surface of the casting will gradually shrink away from the mold liner so that the heat transfer will be across the gap 83 by radiation from the outer surface of the casting skin to the liner 46.

It will be apparent that the temperature gradient between the axis of the casting and its periphery will be greatest at the upper end of the mold. Upon reaching the lower end of the liner 46 the casting will have a substantial skin thickness with an inner annular portion of metal in the mushy stage blending into a molten core 82. It is important at this position to effect a treatment of the casting tending to equalize the tem-

peratures throughout a cross-section of that casting. To accomplish this result the casting is withdrawn through the delayed cooling or temperature equalization zone 63 wherein the sleeve 64 is insulated to substantially eliminate the heat transfer rate between the casting and the cooling water passing between the sleeve 65 and the sleeve 74. Within this zone the molten core 82 of the casting will reheat both the mushy metal 81 and the solid metal portion of the casting and in so giving up its heat the core will gradually become solidified by heat exchange with the skin 80. A sound continuously cast section cannot be made, however, if the molten metal V is excessively long. Therefore, the casting should be embryonic for as short a time as possible.

The pinch rolls 14 shown in Fig. 1 are arranged to engage the casting 13 after it passes through the annular sump tank 75 and to control the speed of withdrawal of the casting from the preceding mold section of the apparatus. The rolls are driven at a controlled constant speed by an electric motor 90 through a conventional speed reducer (not shown) or by other means for effecting a controlled constant speed of casting withdrawal. The rolls are grooved to correspond to the contour of the casting and grip the casting under the influence of a spring or hydraulic pressure sufficient to prevent slippage of the casting.

In the illustrated embodiment of the present invention the apparatus is arranged for the continuous casting of ferrous alloy semi-finished products of circular cross-section. This apparatus is readily adaptable for the production of continuously cast products of other sizes and cross-sectional shapes by corresponding changes in shape of the mold assembly. In addition to the casting of mild steel and alloy steels, the apparatus is adapted for the casting of other high melting point alloys by corresponding changes in the temperature of the molten metal and its rate of pour, the cooling rate, and the speed of casting withdrawal from the apparatus. It is obvious that with the great variety of commercial ferrous alloys and metals in use in industry at the present time, the requirements for the casting of a specific composition of metal will require a particular combination of the casting variables peculiar to that metal composition for the successful continuous casting of commercial products. We have continuously cast the more common ferrous alloys such as mild steel, 18-8, 25-20 and similar alloys successfully in commercial lengths and quantities in an apparatus similar to the one described herein.

Examples of the time-temperature and other relations during typical continuous casting operations with the described apparatus are illustrated in the charts of Figs. 18 and 19. In the charts, the abscissas represent time, in minutes; the left hand ordinates, temperature of metal in degrees F.; and the right hand ordinates power input to the coil of the ladle 11 in kilowatts and the continuous casting rate in feet per minute. The molten metal is tapped from an electric melting furnace and delivered to the holding and pouring ladle 11. This is represented as a time interval *a*—*b* on the charts. The time the molten metal is held in the holding ladle to establish the optimum metal pouring temperature, is represented as the period *b*—*c*. The pouring period for the continuous casting is represented on the charts as the time *c*—*d*. It will be noted that in the run shown in Fig. 18, the molten metal tem-

perature was maintained within a range of plus or minus 10 F. at approximately 2880 F. over a substantial portion of the pouring period. During the last few minutes of the pour the induction heating of the molten metal in the ladle was discontinued but the loss of metal temperature is slight and did not affect the quality of the cast product. The casting was a 4" round of mild carbon steel, 95' in length and its approximate weight 4060 lbs. The withdrawal rate was varied between 2-5 ft./min. In the run illustrated in Fig. 19, the pouring temperature was initially 2820 F. and dropped to 2810 F., and the casting was a 6" round, 25', 5" in length, and its approximate weight 2245 lbs. The casting withdrawal rate was maintained at approximately 1½ ft./min.

As a further example of the operation of the continuous casting apparatus and process in casting a small diameter product, a commercial medium carbon steel having approximately the following composition:

|            | Per cent |
|------------|----------|
| Carbon     | .216     |
| Manganese  | .670     |
| Silicon    | .310     |
| Phosphorus | .016     |
| Sulphur    | .030     |

and the remainder substantially all iron, was melted in an electric furnace and when tapped had a temperature of about 3100 F. During transportation in the transfer ladle 10 the metal cooled so that upon delivery to the ladle 11 its temperature had dropped to approximately 2800 to 2850 F. The actual pouring temperature of the metal entering the mold assembly 12 was in the range of from 2900 to 2950 F., which is a satisfactory temperature for the continuous casting of a metal of this composition. This metal was continuously cast in a mold of circular cross-section with an internal diameter of three inches. With this shape and diameter the casting was pierced in the "as cast" condition, with the necessary reheating. In such a piercing operation, the casting delivered by the continuous casting apparatus was cut into 36 inch lengths for delivery as "tube rounds" to the piercing mill and tubes were produced of, for example, 2½ inch O. D. by ¼ in. wall. Mechanical tests of such tubes indicated in tensile tests an ultimate strength of from 72,000 to 80,000 p. s. i.; a yield point of from 48,000 to 53,000 p. s. i.; and an elongation in two inches of from 35.00 to 37.00 per cent. All samples of such tubes successfully passed the standard A. S. T. M. flattening and flaring tests for this analysis.

In the continuous casting process used to produce these "tube rounds" the mold liner had an internal diameter of three inches with a wall thickness of  $\frac{1}{16}$  inch. Although the mold liner material used in this particular operation was formed of common mild steel, similar results were obtained with a mold liner of the same internal diameter, but formed from a brass tube having a  $\frac{1}{4}$  inch wall thickness and a silver-plated interior surface. With a withdrawal rate of the casting from the mold liner of approximately 48 inches per minute and a co-ordinated molten metal delivery to the top of the mold liner, the water delivery rate through the inlets was approximately 100 gal. per minute at a pressure of 25 p. s. i. This rate of cooling is considered to be lower than is desirable in the commercial practice of the invention. Under these conditions of cool-

ing in the mold, the temperature of the molten metal delivered to the mold was such as to provide approximately 100° F. superheat to assure continuous and controllable metal flow from the pouring ladle.

We have successfully continuously cast carbon steel, for example, in castings of circular or substantially circular cross-section with cooling water supplied in the described manner in volumes ranging from 1.00-2.50 gallons per pound of metal poured into the mold.

The continuous casting formed in the mold moves downwardly below the pinch rolls 14 into the cutting and handling section of the apparatus. This portion of the apparatus, shown in Figs. 1 and 13 to 16 inclusive, is disclosed and claimed in a co-pending application of I. Harter, Jr., and G. A. Pugh, Serial No. 20,738, filed April 13, 1948, now Patent No. 2,582,329 issued January 1, 1952, and includes vertically movable casting cutting provisions, a vertically movable and tilting cradle and a horizontally disposed conveyor. The descending casting moves downwardly into the cradle 91 until its lower end approaches a shelf 98 at the lower end of the cradle and as the downward movement continues is cut to a predetermined length. The shelf is adjustable longitudinally of the cradle to correspond with the length of casting severed. The severed casting 93 drops onto the shelf and the cradle is lowered to a horizontal position from which the casting is removed by the conveyor 94. As soon as the severed casting is removed, the cradle is returned to its upright position to receive the succeeding section of the continuous casting, with the handling process repeated to periodically deliver severed casting lengths to the conveyor 94.

The casting cutting provisions includes a gas cutting torch 92 of the oxy-acetylene type which is mounted on a carriage 95 which is arranged for vertical movements within predetermined limits between the pinch rolls 14 and the cradle 91. As shown in Figs. 13, 14 and 15, the carriage 95 is arranged for vertical movement guided by wheels 96 on spaced channel irons 97. The upper portion of the carriage has a pair of pivoted jaws 100 operated by a double-acting power cylinder 103 through a linkage 102 and common pivot pin 101 to grip the continuous casting 13 so that the carriage and the torch will move downwardly with the casting. When the casting has been cut to a predetermined length, the jaws gripping the casting are released and the carriage returned to its upper position to repeat the cutting operation. A plate 104 having two spaced depending flanges 105 embracing the body of the torch 92 is supported by a pair of spaced pivots 106, each of which includes a rotatable pin 107 secured to the plate 104 and having a clevis 110 at its upper end. The clevis is fitted with a bolt 111 extending through a horizontal slot in an arm 112 which in turn forms the lower end of a second rotatable pin 113 mounted upon the carriage 95. A worm 114 in bearings 115 slideably mounted in the frame of the carriage 95 is arranged to engage a correspondingly threaded sleeve 116 attached to the plate 104 and is turned by a handwheel 117. Thus, the handwheel regulates the movement of the torch 92 whereby the torch flame may be moved in a horizontal plane to traverse the casting 13.

The cradle 91 of the handling portion 15 of the continuous casting apparatus is shown in Figs. 1 and 16. In Fig. 16 the cradle is shown with a severed casting 93 supported therein in an up-

right position (shown in solid lines) immediately after the casting has been severed by the torch 92; in an intermediate position (shown in dot-dash lines); and in a horizontal position (shown in dotted lines) immediately prior to the removal therefrom of the severed casting by the conveyor 94. The cradle 91 is formed by a pair of channel members arranged back to back to form opposite sides thereof and spaced apart by a set of longitudinally spaced transverse channels extending across the bottom 123 of the cradle. The spaced transverse channels provide openings therebetween matching the rolls of the conveyor 94 when the cradle is in its horizontal position. The top side 124 of the cradle is open whereby the cradle may be returned to its upright position after delivering one severed casting, without interfering with the withdrawal of the succeeding section of the continuous casting 13.

20 The cradle 91 is guided in its movement between a vertical and horizontal position by a pair of flanged wheels 125 mounted on the bottom 123 at a location near one end, and by a pair of flanged wheels 127 mounted on the top side 124 at 25 the opposite end of the cradle. The movement of the wheels 125 is confined to a vertical direction by guide rails, but since the gage of those wheels is greater than the width of the cradle, the cradle is free to pivot about the wheel axis in its downward movement. The movement of the wheels 127 is directed by a spaced pair of rails 132 which extend vertically a short distance and are bent in a short radius 90° bend to extend horizontally a distance substantially equal to the longitudinal 35 distance between the axis of wheels 125 and 127.

The severed casting 93 and its supporting cradle 91 are lowered from the upright position by an electrically-driven drum hoist 133 equipped with dynamic braking and connected to the cradle by a pair of cables 134. The cables pass over a pair of sheaves 135 rotatable on the structural framework supporting the continuous casting apparatus.

After the continuous casting has been severed by the torch 92, the downward movement of the cradle is immediately initiated by starting the motor-driven drum hoist 133. The severed casting 93 is forced toward the bottom 123 of the cradle and held in that position until the outward swing of the upper end of the cradle, as determined by the guide wheels 125 and 127, has progressed to a point whereby the weight of the casting will hold it in position against the bottom of the cradle. This is accomplished by a power piston 136 supported on the framework of the continuous casting apparatus which forces the severed casting toward the bottom 123 to rest against the transverse channels. The action of the piston is controlled by limit switches (not shown) allowing it to push only when the cradle is near its vertical position.

The conveyor 94 includes a series of circumferentially grooved motor-driven rollers 142, with the individual rollers spaced to match corresponding openings in the bottom 123 of the cradle 91. Due to the necessity for speed in lowering the cradle, discharging the severed casting and returning the cradle into position for a subsequent section of casting, the lowering mechanism is provided with a shock absorbing device 143 positioned between the rollers 142 of the conveyor 94 adjacent one end of the cradle when it is in its horizontal position.

The shock absorbing device includes a pneumatically operated arm which contacts a project-

tion 155 on the cradle 91. Contact between the device 143 and the cradle projection 155 is attained as the cradle approaches its horizontal position with the downward movement of the cradle arrested by a progressively increasing force created pneumatically which brings the cradle to a stop without appreciable shock in contacting the rollers 142 with the casting 93.

With the described process and apparatus, the length of the continuous casting produced will depend primarily upon the metal holding capacity of the ladle 11 and the speed at which its molten metal content can be replenished. When the ladle is exhausted or for any reason the pouring operation is temporarily discontinued, a metal bolt is inserted into the top of the casting in the mold with its head projecting, to serve as a substitute for the dummy bolt 163 when pouring is resumed, thus avoiding complete removal of the casting and reinsertion of the dummy 164.

The described continuous casting process and apparatus will result in a substantial reduction in the cost of production of small dimensional shapes of ferrous alloys and other high fusion temperature metals due to the substantial elimination of cropping and scalping losses inherent in individual stationary mold casting and also due to the elimination of the time and equipment required for heat treating and reducing the blooms to the size range of the continuous cast product. While the quality of the cast ferrous alloy products, with respect to the possibility of porous centers or center cracks, tends to decrease, particularly with the larger diameter castings, as the casting speed is increased, castings with such defects have been found to be commercially acceptable for a wide range of ferrous alloy products. With slower casting speeds and/or smaller diameter castings, the quality of the product has been equal, if not superior, to the steel and alloy steel rounds or billets now used for seamless tube manufacture.

While in accordance with the provisions of the statutes we have illustrated and described herein the best form and mode of operation of the invention now known to us, those skilled in the art will understand that changes may be made in the form of the process and apparatus disclosed without departing from the spirit of the invention covered by our claims, and that certain features of our invention may sometimes be used to advantage without a corresponding use of other features.

We claim:

S

1. The method of continuously casting molten ferrous metals and alloys in an open-ended vertical mold having a laterally confined space around the mold wall outer surface for the flow of a liquid coolant and including a movable dummy bottom to which the casting formed in the mold initially attaches, which comprises delivering the molten metal to be cast into the upper end of the mold, maintaining a non-wetting heat transfer contact between the molten metal in the mold and the mold wall inner surface continuously introducing cooling water at a substantial superatmospheric pressure into the laterally confined space around the mold wall outer surface at a level therein above the normal maximum level of molten metal in the mold and passing the cooling water downwardly through said space at a velocity insuring a highly turbulent cooling water flow in contact with said mold wall outer surface at the level of molten metal in the mold.

and in quantities of at least one gallon of cooling water per pound of ferrous metal cast, insuring a rate of heat transfer through the mold wall sufficient to cause a rapid progressive formation of a casting shell around the mass of molten metal in the mold, and withdrawing the dummy bottom and embryo casting formed thereon downwardly from the bottom of the mold.

2. The method of continuously casting molten ferrous metals and alloys in an open-ended vertical mold having a laterally confined space around the mold wall outer surface for the flow of a liquid coolant, said mold being formed of metal having a melting temperature below the temperature of the metal to be cast and including a movable dummy bottom to which the casting formed in the mold initially attaches, which comprises continuously delivering the molten metal to be cast into the upper end of the mold, continuously maintaining a non-wetting heat transfer contact between the mass of molten metal in the mold and the mold wall inner surface while continuously introducing cooling water at a substantial superatmospheric pressure into the laterally confined space around the mold wall outer surface at a level therein above the normal maximum level of molten metal in the mold and passing the cooling water downwardly through said space at a velocity insuring a highly turbulent cooling water flow in contact with said mold wall outer surface at the level of molten metal in the mold and in quantities of at least one gallon of cooling water per pound of ferrous metal cast, insuring a rate of heat transfer through the mold wall sufficient to cause a rapid progressive formation of a casting shell around the mass of molten metal in the mold, and withdrawing the dummy bottom and embryo casting formed thereon downwardly from the bottom of the mold.

3. The method of continuously casting molten ferrous metals and alloys in an open-ended vertical mold having a laterally confined space around the mold wall outer surface for the flow of a liquid coolant and including a movable dummy bottom to which the casting formed in the mold initially attaches, which comprises delivering the molten metal to be cast into the upper end of the mold, maintaining a non-wetting heat transfer contact between the mass of molten metal in the mold and the mold wall inner surface, continuously introducing cooling water at a substantial superatmospheric pressure into the laterally confined space around the mold wall outer surface at a level therein above the normal maximum level of molten metal in the mold and passing the cooling water downwardly through said space at a velocity of at least 40 feet per second insuring a highly turbulent cooling water flow in contact with said mold wall outer surface at the level of molten metal in the mold and in quantities of at least one gallon of cooling water per pound of ferrous metal cast, insuring a rate of heat transfer through the mold wall sufficient to cause a rapid progressive formation of a casting shell around the mass of molten metal in the mold, and withdrawing the dummy bottom and embryo casting formed thereon downwardly from the bottom of the mold.

4. The method of continuously casting molten ferrous metals and alloys in an open-ended vertical mold having a laterally confined space around the mold wall outer surface for the flow of a liquid coolant and including a movable dummy bottom to which the casting formed in

the mold initially attaches, which comprises delivering the molten metal to be cast into the upper end of the mold, maintaining a non-wetting heat transfer contact between the mass of molten metal in the mold and the mold wall inner surface while continuously introducing cooling water at a substantial superatmospheric pressure into the laterally confined space around the mold wall outer surface at a level therein above the normal maximum level of molten metal in the mold and passing the cooling water downwardly through said space at a velocity insuring a highly turbulent cooling water flow in contact with said mold wall outer surface at the level of molten metal in the mold and in quantities of at least one gallon of cooling water per pound of ferrous metal cast, insuring a rate of heat transfer through the mold wall sufficient to cause a rapid progressive formation of a casting shell around the mass of molten metal in the mold, discharging the cooling water from the laterally confined space around the mold wall outer surface directly into a zone of atmospheric pressure, and withdrawing the dummy bottom and embryo casting formed thereon downwardly from the bottom of the mold.

5. The method of continuously casting molten ferrous metals and alloys in an open-ended vertical mold having a laterally confined space around the mold wall outer surface for the flow of a liquid coolant, said mold being formed of metal having a melting temperature below the temperature of the metal to be cast and including a movable dummy bottom to which the casting formed in the mold initially attaches, which comprises continuously delivering the molten metal to be cast into the upper end of the mold, continuously maintaining a non-wetting heat transfer contact between the mass of molten metal in the mold and the mold wall inner surface while continuously introducing cooling water at a substantial superatmospheric pressure into the laterally confined space around the mold wall outer surface at a level therein above the normal maximum level of molten metal in the mold and passing the cooling water downwardly through said space at a velocity of at least 40 feet per second insuring a highly turbulent cooling water flow in contact with said mold wall outer surface at the level of molten metal in the mold and in quantities of at least one gallon of cooling water per pound of ferrous metal cast, insuring a rate of heat transfer through the mold wall sufficient to cause a rapid progressive formation of a casting shell around the mass of molten metal in the mold, discharging the cooling water from the lower end of the laterally confined space around the mold wall outer surface directly into a zone of atmospheric pressure, and withdrawing the dummy bottom and embryo casting formed thereon downwardly from the bottom of the mold.

6. The method of continuously casting molten ferrous metals and alloys in an open-ended vertical mold having a laterally confined space around the mold wall outer surface for the flow of a liquid coolant, said mold being formed of metal having a melting temperature below the temperature of the metal to be cast and including a movable dummy bottom to which the casting formed in the mold initially attaches, which comprises delivering the molten metal to be cast into the upper end of the mold, continuously maintaining a non-wetting heat transfer contact between the mass of molten metal in the mold and

the mold wall inner surface, continuously introducing cooling water at a substantial superatmospheric pressure and in a solid stream into the laterally confined space around the mold wall outer surface at a level therein above the normal maximum level of molten metal in the mold and passing the cooling water downwardly through said space at a velocity of at least 40 feet per second, insuring a highly turbulent cooling water flow in contact with said mold wall outer surface at the level of molten metal in the mold and a rate of heat transfer through the mold wall sufficient to cause a rapid progressive formation of a casting shell around the mass of molten metal in the mold, and withdrawing the dummy bottom and embryo casting formed thereon downwardly from the bottom of the mold.

7. The method of continuously casting molten ferrous metals and alloys in an open-ended vertical mold having a laterally confined space around the mold wall outer surface for the flow of a liquid coolant, said mold being formed of metal having a melting temperature below the temperature of the metal to be cast and including a movable dummy bottom to which the casting formed in the mold initially attaches, which comprises delivering the molten ferrous metal to be cast into the upper end of the mold, continuously maintaining a non-wetting heat transfer contact between the mass of molten metal in the mold and the mold wall inner surface, continuously introducing cooling water at a substantial superatmospheric pressure and in a solid stream into the upper end of the laterally confined space around the mold wall outer surface and accelerating the cooling water downwardly through said space at a velocity of at least 40 feet per second, insuring a highly turbulent cooling water flow in contact with said mold wall outer surface at the level of molten metal in the mold and a rate of heat transfer through the mold wall sufficient to cause a rapid progressive formation of a casting shell around the mass of molten metal in the mold, discharging the cooling water from the lower end of the laterally confined space around the mold wall outer surface directly into a zone of atmospheric pressure, and withdrawing the dummy bottom and embryo casting formed thereon downwardly from the bottom of the mold.

8. The method of continuously casting molten ferrous metals and alloys in an open-ended vertical mold having a laterally confined space around the mold wall outer surface for the flow of a liquid coolant, said mold being formed of metal having a melting temperature below the temperature of the metal to be cast and including a movable dummy bottom to which the casting formed in the mold initially attaches, which comprises continuously delivering the molten metal to be cast through an oxidizing atmosphere into the upper end of the mold above the molten level therein, maintaining a non-oxidizing atmosphere and an oxide-free molten metal surface in the mold by continuously introducing a non-oxidizing gas into the upper end of said mold above the molten metal level therein and supplying a liquid hydrocarbon to the mold wall inner surface above the molten metal level in the mold, continuously introducing cooling water at a substantial superatmospheric pressure into the laterally confined space around the mold wall outer surface at a level therein above the normal maximum level of molten metal in the mold and passing the cooling water downwardly through said space at a velocity of at least 40 feet per second, insuring

a highly turbulent cooling water flow in contact with said mold wall outer surface at the level of molten metal in the mold and in quantities insuring a rate of heat transfer through the mold wall sufficient to cause a rapid progressive formation of a casting shell around the mass of molten metal in the mold, and withdrawing the dummy bottom and embryo casting formed thereon downwardly from the bottom of the mold.

9. Continuous casting apparatus comprising a mold assembly including an open-ended stationary upright vertically elongated tubular mold liner formed of high thermal conductivity metal, an open-ended vertically elongated tubular member at the outer side of said mold liner and cooperating therewith to form a peripheral cooling liquid passage therebetween opening at its lower end directly to a zone of atmospheric pressure, means for supporting said mold liner and tubular member at their upper ends only, whereby their lower end are free to expand and contract, and means for supplying cooling liquid to the upper end of said passage comprising means arranged to form a cooling liquid supply chamber surrounding the upper portions of said mold liner and tubular member and means arranged to form a progressively converging cooling liquid entrance section connecting the upper part of said supply chamber to the upper end of said passage.

10. Continuous casting apparatus comprising a mold assembly including an open-ended stationary upright vertically elongated tubular mold liner formed of high thermal conductivity metal, an open-ended vertically elongated tubular skirt member coaxial with and surrounding said mold liner and uniformly spaced therefrom to form a narrow peripheral cooling liquid passage therebetween of uniform cross-sectional area throughout its extent and opening at its lower end directly to a zone of atmospheric pressure, means for supporting said mold liner and skirt member at their upper ends only, whereby their lower ends are free to expand and contract, and means for supplying cooling liquid to the upper end of said passage comprising means arranged to form a downwardly tapering annular cooling liquid entrance section having its lower end opening to the upper end of said passage.

11. Continuous casting apparatus comprising a mold assembly including an open-ended stationary upright vertically elongated tubular mold liner formed of high thermal conductivity metal and of uniform cross-sectional area throughout its length, an open-ended vertically elongated tubular skirt member coaxial with and surrounding said mold liner and uniformly spaced therefrom to form a narrow peripheral cooling liquid passage therebetween of uniform cross-sectional area throughout its extent and opening throughout the entire periphery of its lower end directly to a zone of atmospheric pressure, means for supporting said mold liner and skirt member at

their upper ends only, whereby their lower ends are free to expand and contract, and means for supplying cooling liquid to the upper end of said passage comprising means arranged to form a cooling liquid supply chamber surrounding the upper end portions of said mold liner and skirt member and means arranged to form a downwardly tapering annular cooling liquid entrance section connecting the upper part of said supply

- 10 chamber to the upper end of said passage.
12. Continuous casting apparatus comprising a mold assembly including an open-ended stationary upright vertically elongated tubular mold liner formed of high thermal conductivity metal and of uniform cross-sectional area throughout its length, an open-ended vertically elongated tubular skirt member coaxial with and surrounding said mold liner and uniformly spaced therefrom to form a narrow peripheral cooling liquid passage therebetween of uniform cross-sectional area throughout its extent and opening throughout the entire periphery of its lower end to a zone of atmospheric pressure, means for supporting said mold liner and skirt member at their upper ends only, whereby their lower ends are free to expand and contract, means for supplying cooling liquid to the upper end of said passage comprising means arranged to form a cooling liquid supply chamber surrounding the upper 15 end portions of said mold liner and skirt member and means arranged to form a downwardly tapering annular cooling liquid entrance section connecting the upper part of said supply chamber to the upper end of said passage, and deflector means on said mold liner below the lower end of said skirt member arranged to deflect outwardly cooling liquid discharged from the lower end of said passage.

ISAAC HARTER.

ISAAC HARTER, JR.

OTIS R. CARPENTER.

#### REFERENCES CITED

The following references are of record in the file of this patent:

#### UNITED STATES PATENTS

| Number       | Name             | Date          |
|--------------|------------------|---------------|
| 894,410      | Trotz            | July 28, 1908 |
| 50 1,503,479 | Coats            | Aug. 5, 1924  |
| 1,894,982    | Eppenstein       | Jan. 24, 1933 |
| 2,079,644    | Williams         | May 11, 1937  |
| 2,163,967    | Strawn et al.    | June 27, 1939 |
| 2,184,519    | Eppenstein       | Dec. 26, 1939 |
| 55 2,187,720 | Williams         | Jan. 23, 1940 |
| 2,206,888    | Greenidge        | July 9, 1940  |
| 2,264,287    | Betterton et al. | Dec. 2, 1941  |
| 2,284,704    | Welblund         | June 2, 1942  |
| 2,290,083    | Webster          | July 14, 1942 |
| 60 2,304,258 | Junghans         | Dec. 8, 1942  |
| 2,357,780    | Mueller          | Sept. 5, 1944 |
| 2,376,518    | Spence           | May 22, 1945  |
| 2,509,079    | Trewin et al.    | May 23, 1950  |